

## UNITED STATES PATENT OFFICE.

CONRAD KÖRTLING AND CARL JAENTSCH, OF CASSEL, GERMANY.

## MANUFACTURE OF BUILDING-BLOCKS.

957,351.

Specification of Letters Patent. Patented May 10, 1910.

No Drawing.

Application filed April 1, 1909. Serial No. 487,295.

*To all whom it may concern:*

Be it known that we, CONRAD KÖRTLING and CARL JAENTSCH, both subjects of the German Emperor, and residents of 3 Hedwigstrasse and 37 Webergstrasse, respectively, Cassel, Germany, have invented certain new and useful Improvements in the Manufacture of Building-Blocks, of which the following is a specification.

10 This invention relates to the manufacture of building blocks from peat.

Hitherto bricks have been made by reducing peat to a pulp or to fibers and adding agglutinants so as to form a moldable mass from which the bricks are molded, the whole being closely united by pressure. Peat has also been rendered fit for many useful purposes by submitting it to a steeping process in compositions adapted to render it elastic and fireproof. It has also been pressed and dried and mixed with water-glass and then further compressed so as to form a hard material out of which boxes can be made.

According to the present invention, building blocks are made by impregnating unpressed pieces of peat with a solution of water-glass, and according to another phase of the invention, building blocks are made from unpressed pieces of peat by coating them with a layer of any suitable fire-proofing material, the central portion of the peat remaining unaltered. Water-glass may be employed to form this coating.

According to the first phase of the invention, the peat, which is cut directly out of the soil without being pressed or molded, is saturated, after being dried, with a solution of water-glass and the peat is then allowed to dry. This solution of water-glass may vary. Thus, soda water-glass, potash water-glass or potash lime water-glass (which is a mixture of potash water-glass and lime) may be used, the latter being the most resisting. When said latter material is employed the blocks can be used with particular advantage for brick-work very close to hot objects, such as bakers' ovens.

According to the second part of the invention the unpressed peat is simply coated with any suitable fire-proofing material, such as water-glass. Blocks so made may be used for walls having to carry no weight.

For making walls of blocks or bricks made in either way any kind of mortar may be

used, but a mixture of water-glass with a 55 hydraulic material, such as Roman or Portland cement, is particularly suitable, as by the same a close union of the bricks coated or saturated with a solution of water-glass is effected.

A wall made of these bricks is a perfect substitute for any loam or plaster wall or wall formed of plaster of paris with reinforcing wire-work, and nails can be driven into it; and it has moreover the advantage of not conducting sound and of being a bad conductor of heat, as the brick remains porous. A further and very important advantage is that bricks thus impregnated are fire-proof and are not destroyed even under the 70 influence of the greatest heat. Such bricks are particularly suitable for outside walls of small one-storied buildings as they are not affected by the weather. But partition 75 walls and floors or ceilings, and especially intermediate layers in ceilings and walls, can also be made with them very advantageously. They can likewise be used for making building plates or slabs of a rather large size, as their weight is exceedingly small.

What we claim is:—

1. A process of manufacturing building blocks, which comprises the impregnation of unpressed blocks of peat with a solution of water-glass.

2. A process of manufacturing building blocks, which comprises coating unpressed blocks of peat with a layer of water-glass, the central portion of the peat block remaining unaltered.

3. A building block consisting of an unpressed block of peat impregnated with water-glass.

4. A building block consisting of an unpressed block of peat provided with a coating of fire-proofing material, the central portion of the block remaining in its natural condition.

In testimony whereof we have hereunto signed our names this 22d day of March 100 1909, in the presence of two subscribing witnesses.

CONRAD KÖRTLING.  
CARL JAENTSCH.

Witnesses:

EMANUEL SCMERZ,  
ERNST KRESST.